

1

3,168,385  
MOTOR FUELS

John J. Giammaria and Henry D. Norris, Woodbury, N.J., assignors to Socony Mobil Oil Company, Inc., a corporation of New York  
No Drawing. Filed July 12, 1961, Ser. No. 123,419  
6 Claims. (Cl. 44—56)

The present invention relates to new and improved fuel compositions having a relatively high octane number and, more particularly, to such compositions containing anti-knock additives and other addition agents that further improve, or appreciate, the anti-knock qualities thereof.

As is well known to those skilled in the art, octane level requirements for gasolines have been steadily rising to a level that approaches 100 O.N. and higher. To some extent, octane requirements have been met by special refining methods, such as catalytic reforming. Higher octane numbers have also been achieved by the addition of anti-knock agents. In order to achieve octane ratings in the order of 100 O.N., however, resort has been made to a combination of reforming plus addition of an anti-knock agent. If further octane improvement or appreciation is required, severe reforming can be used, but it is very expensive. Another alternative is to increase the amount of anti-knock agent but, in the case of many anti-knock agents, such as tetraethyl lead, additional amounts give less octane improvement per incremental amount. Thus, being expensive, such usage of lead-containing anti-knock agents for obtaining octane numbers in the order of 100 or more is at a high cost per octane number.

It has been proposed to increase the octane rating of certain gasolines by adding relatively inexpensive materials to a fuel containing anti-knock agents so as to increase the octane rating without using additional expensive anti-knock agent. Such materials, which for convenience herein are called anti-knock "appreciators," include esters of weak organic carboxylic acids as disclosed in British Patent No. 866,610. In that patent, it is disclosed that the esters of weak carboxylic acids, such as t-butyl acetate, appreciate the octane number of certain leaded gasolines that must contain at least 10% aromatic and/or olefin content in order for the appreciator to be effective. Otherwise, and as to a gasoline consisting essentially of saturated aliphatic hydrocarbons, the appreciators disclosed in the British patent are specifically set forth as having no effect on octane improvement even though a lead anti-knock agent is present. As is more specifically shown in the British patent, in Table V thereof, an isobutane-isobutylene alkylate containing 3 cc./U.S. gallons of TEL was not affected by use of t-butyl acetate as an octane appreciator.

It has now been found that in a motor fuel in the gasoline boiling range (e.g., about 75° F. to about 450° F.) consisting essentially of saturated aliphatic hydrocarbons and a small but anti-detonant amount of tetraethyl lead, the alkyl esters of weak organic monocarboxylic acids appreciate the octane number of the lead-containing saturated aliphatic hydrocarbon fuel if a dialkyl ether is blended with the fuel. Such a discovery is not only a marked improvement in that it enables obtainment of octane appreciation with leaded base stocks (saturated aliphatic hydrocarbons) for which the art has shown ineffective results with the alkyl esters of weak monocarboxylic acids but, of considerable importance, the present invention enables the production of leaded motor fuels, based on saturated aliphatic hydrocarbons, that can be appreciated to octane numbers of at least 100 and to even 110 or more by use of alkyl esters of weak monocarboxylic acids as appreciators. As is shown more fully hereinafter, practice of this invention enables the provi-

2

sion of such exceptionally high octane number gasolines by use of TEL-containing blend of a saturated aliphatic hydrocarbon base stock (e.g., alkylate) and a dialkyl ether, the octane number of which blend is appreciated by an alkyl ester of a weak organic monocarboxylic acid. Moreover, and as is apparent from the herein-described invention, it enables the provision of motor fuels of exceptionally high octane number from saturated aliphatic hydrocarbons without requirements for presence of high octane components of the aromatic- and olefinic-type hydrocarbons.

In reference to the saturated aliphatic hydrocarbon base stock of the novel fuel embodied herein, particularly suitable are hydrocarbon fractions in the gasoline boiling range that are composed or substantially composed of branched chain saturated aliphatic hydrocarbons and, preferably, have a high octane number, such as in the order of a clear octane number of at least 80, and more preferably, 90 or more. Particularly suitable for practice of this invention are the so-called "alkylates," known to those skilled in the art, that are mainly composed of highly branched paraffins such as, highly branched octanes, highly branched heptanes, highly branched nonanes, mixtures thereof, and others. Such alkylates can be prepared by any of several methods known to those skilled in the art, inclusive of which are the alkylation of isobutane with butylenes, alkylation of isoamylene with propenes, and the like, by processes using alkylation catalysts such as sulfuric acid, hydrofluoric acid and others. Thus as used herein, the term "alkylate" includes not only compositions of branched chain paraffins as aforesaid, but also 2, 3, 4-trimethylpentane, commercial isoctanes comprising primarily trimethylpentanes and, more specifically, alkylate produced by commercial methods by alkylation of isobutane with butylene and, still more specifically, such an alkylate having a research octane number (clear) of at least 80 and boiling in the gasoline boiling range.

The ether component of the fuel compositions embodied herein are the dialkyl ethers of the formula



wherein R and R' are the same or different alkyl radicals and which boil at a temperature in the boiling range of gasoline. For use in practice of this invention, the stated ethers should contain a total of at least four as the sum of the carbon atoms in the two alkyl groups and, desirably, not more than 10. Examples of such ethers include diisopropyl ether, t-butyl methyl ether, di-n-propyl ether, amyl ethyl ether, t-butyl ethyl ether, and the like.

As aforesaid, the novel compositions embodied herein contain tetraethyl lead as the anti-knock agent, but if desired, other lead-containing anti-knock agents may be present in addition to the tetraethyl lead. Examples of such other lead-containing anti-knock agents include tetramethyl lead and tetrapropyl lead.

The anti-knock appreciators contemplated for use in practice of this invention are t-alkyl esters of weak organic monocarboxylic acids; more particularly, the tertiary alkyl esters of aliphatic monocarboxylic acids of two to eight carbon atoms, as for example, the tertiary alkyl esters of acids such as acetic acid, propionic acid, caproic acid, 2-ethyl hexanoic acid, and the like; and still more specifically, such esters of saturated aliphatic hydrocarbon monocarboxylic acids of from two to four carbon atoms; and the tertiary alkyl esters of benzoic acid. As to the tertiary alkyl group of the esters embodied for use herein, examples thereof include t-butyl, t-amyl, t-octyl and more specifically, a t-alkyl group of four to eight carbon atoms. Thus, specific embodiments of such esters include t-butyl acetate, t-amyl caproate, t-octyl acetate, t-butyl benzoate, and the like. Particularly preferred for practice of this invention are the t-butyl

esters of the lower molecular weight saturated aliphatic hydrocarbon monocarboxylic acids of two to four carbon atoms and, for example, t-butyl acetate.

In general, the compositions of this invention comprise a saturated aliphatic hydrocarbon base stock in the gasoline boiling range blended with an ether, as afore-defined, in which the base stock may comprise from about 50% to about 95% by volume of the blend, tetraethyl lead in a small amount sufficient to increase the anti-knock characteristics of the blend, and preferably from about one to about four milliliters of tetraethyl lead per gallon of the blend, and a small amount, sufficient to appreciate the octane number of such a lead-containing blend, of an octane appreciator as hereinbefore defined. More specifically, the appreciator is used in an amount of from about one to about 50 grams, and still more preferably, about five to about 25 grams per gallon of the blend.

In order to further describe the invention, the following tabulation contains several embodiments of this invention as well as, for comparison purposes, comparable compositions but in which a dialkyl ether or tetraethyl lead was not used. The unexpected improvement in octane appreciation by use of a dialkyl ether-alkylate blend containing both TEL (tetraethyl lead) and the octane appreciators is evident from the extent of octane increase shown in the tabulation for the embodiments of this invention. It has been found, statistically, that the R.O.N. can vary somewhat at the high octane level from test to test, and that an O.N. improvement of at least 0.6 O.N. in duplicate tests was necessary to be significant. Accordingly, an appreciator that does not appreciate O.N. by at least 0.6 O.N. or more is not considered to be effective.

The base stock used for the composition of the examples in the tabulation was an isobutane-butylene alkylate having a Reid Vapor Pressure of 7.5 lbs. and the following distillation points: 10% at 150° F., 50% at 216° F., 90% at 236° F. and an end boiling point of 305° F.

poses of illustration by use of the novel combination of the defined hydrocarbon base stock-dialkyl ether blend, tetraethyl lead and an appreciator, the compositions embodied herein may contain other additives designed to impart other improved properties. Thus, the compositions may contain anti-rust agents, metal deactivators, dyes, anti-oxidants, detergents, etc.

Although the present invention has been described with preferred embodiments, it is to be understood that modifications and variations may be resorted to, without departing from the spirit and scope of this invention, as those skilled in the art will readily understand. Such variations and modifications are considered to be within the purview and scope of the appended claims.

What is claimed is:

1. A motor fuel blend of from about 50 to about 95% by volume of a saturated aliphatic hydrocarbon base stock in the gasoline boiling range and from about 5 to about 50% of a dialkyl ether containing from 4 to 10 as the sum of the carbon atoms in the two alkyl groups, containing a small amount, sufficient to increase the anti-knock characteristics of said blend, of tetraethyl lead, and from about one to about fifty grams, per gallon of said blend and sufficient to appreciate the octane number of said blend containing the tetraethyl lead, of a tertiary C<sub>4</sub> to C<sub>8</sub> alkyl ester of a C<sub>2</sub> to C<sub>8</sub> organic monocarboxylic hydrocarbon acid.

2. A motor fuel, as defined in claim 1, wherein the saturated aliphatic hydrocarbon base stock has a Research Octane Number of at least 80, the tetraethyl lead is present in an amount of from about one to about four milliliters per gallon of the blend of base stock and ether, and the tertiary alkyl ester of an organic monocarboxylic acid is present in an amount of from about one to about fifty grams per gallon of said blend.

3. A motor fuel, as defined in claim 1, wherein the tertiary alkyl ester of an organic monocarboxylic acid is a tertiary C<sub>4</sub> to C<sub>8</sub> alkyl ester of a C<sub>2</sub> to C<sub>8</sub> saturated aliphatic hydrocarbon monocarboxylic acid.

4. A motor fuel, as defined in claim 1, wherein the

| Example Number | Percent Ether in Alkylate (by volume) | Anti-Knock Agent (grams/gal. of Pb as TEL or TML) <sup>2</sup> | Research Octane No. of Base Fuel | Octane Appreciator, 25.0 g./gal. | Research Octane No. <sup>1</sup> Increase with Appreciator |
|----------------|---------------------------------------|----------------------------------------------------------------|----------------------------------|----------------------------------|------------------------------------------------------------|
| 1-----         | None-----                             | None-----                                                      | 93.0                             | t-Butyl acetate-----             | 0.0                                                        |
| 2-----         | do-----                               | 3.18 (TEL) <sup>3</sup>                                        | 102.0                            | do-----                          | 0.4                                                        |
| 3-----         | do-----                               | 3.18 (TML) <sup>3</sup>                                        | 102.0                            | do-----                          | -0.5                                                       |
| 4-----         | 20% diisopropyl ether                 | 3.18 (TML)                                                     | 106.5                            | do-----                          | -0.7                                                       |
| 5-----         | do-----                               | 3.18 (TEL)                                                     | 108.7                            | do-----                          | 1.5                                                        |
| 6-----         | 10% diisopropyl ether                 | 3.18 (TEL)                                                     | 105.5                            | do-----                          | 1.4                                                        |
| 7-----         | 10% t-butyl methyl ether              | 3.18 (TEL)                                                     | 109.2                            | do-----                          | 0.7                                                        |
| 8-----         | 20% t-butyl methyl ether              | 3.18 (TEL)                                                     | 112.5                            | t-butyl benzoate (12.5 g./gal.)  | 1.2                                                        |

<sup>1</sup> A.S.T.M. Research Method (D-908).

<sup>2</sup> TEL=Tetraethyl Lead.

<sup>3</sup> TML=Tetramethyl Lead.

As is apparent from the data in the foregoing tabulation, the octane appreciator (t-butyl acetate) had no effect on the Research Octane Number of a composition consisting of the alkylate and the appreciator (Ex. 1). Neither did the appreciator have any significant effect on Research Octane Number in the same composition (Ex. 2) but which contained TEL (tetraethyl lead); nor did the appreciator increase, but actually decreased the octane number in alkylate (Ex. 3) and an alkylate-ether blend (Ex. 4) containing TML as the sole anti-knock agent. However, as shown for Ex. Nos. 5-8, inclusive, for the compositions containing the component combination of this invention (alkylate-ether, TEL and the defined appreciators), the appreciator substantially increased the octane number even at the high octane levels shown for the base fuel.

Although the invention has been described for pur-

60 tertiary alkyl ester of an organic monocarboxylic hydrocarbon acid is a t-alkyl ester of benzoic acid in which the t-alkyl group contains four to eight carbon atoms.

65 5. A motor fuel, as defined in claim 1, wherein the base stock is an alkylate, the ether is a member from the group consisting of diisopropyl ether and t-butyl methyl ether, and the tertiary alkyl ester of an organic monocarboxylic hydrocarbon acid is a member from the group consisting of t-butyl acetate and t-butyl benzoate.

70 6. A motor fuel blend, by volume, of from about 50 to about 95% of an alkylate in the gasoline boiling range from about 5 to about 50% of a dialkyl ether from the group consisting of diisopropyl ether and t-butyl methyl ether, said alkylate having a Research Octane Number of at least 80 clear, from about one to about four milliliters of tetraethyl lead per gallon of said blend, and from about one to about fifty grams, per gallon of said

blend, of an ester from the group consisting of t-butyl acetate and t-butyl benzoate.

References Cited in the file of this patent

UNITED STATES PATENTS

|           |                  |                |
|-----------|------------------|----------------|
| 2,046,243 | Buc              | June 30, 1936  |
| 2,209,204 | McCulloch et al. | July 23, 1940  |
| 2,210,942 | Lipkin           | Aug. 13, 1940  |
| 2,334,006 | Holm             | Nov. 9, 1943   |
| 2,384,866 | Wiczer           | Sept. 18, 1945 |

5 504,837

2,409,746  
3,009,793

Evans et al. Oct. 22, 1946  
Eckert et al. Nov. 21, 1961

FOREIGN PATENTS

Great Britain May 2, 1939

OTHER REFERENCES

"Improved Motor Fuels Through Selective Blending,"  
by Wagner et al., paper presented at 22nd Annual Meeting of American Petroleum Institute, November 7, 1941;  
19 pages.